

April 3, 1962

R. OWEN

3,028,255

HEAT-SENSITIVE COPY-SHEET

Filed Oct. 26, 1959



INVENTOR  
RICHARD OWEN

by  
Carpenter, Abbott, Coulter + Kinney  
ATTORNEYS

# United States Patent Office

3,028,255

Patented Apr. 3, 1962

1

3,028,255

## HEAT-SENSITIVE COPY-SHEET

Richard Owen, Brooklyn Center, Minn., assignor to Minnesota Mining and Manufacturing Company, St. Paul, Minn., a corporation of Delaware

Filed Oct. 26, 1959, Ser. No. 848,550

11 Claims. (Cl. 117—36.8)

This application is a continuation-in-part of my co-pending application Serial No. 594,540, filed June 28, 1956, now Patent No. 2,910,377.

This invention relates to heat-sensitive copy-paper useful in the thermographic reproduction of differentially radiation-absorptive graphic originals as described in Miller United States Patent No. 2,740,896 and employing apparatus such as described in Miller United States Patent No. 2,740,895 or in Kuhrmeyer et al. United States Patent No. 2,891,165. In particular, the invention relates to thermographic heat-sensitive copy-paper in which the required visible change results from inter-reaction involving, for example, such inter-reactants as organic amine molybdates and organic reducing agents. In a preferred form the invention provides white copy-sheets, which when suitably heated, as in the thermographic copying process, yield images in a variety of colors depending on the specific components employed. A non-fading copy is thus directly produced, without any subsequent processing such as developing, fixing, washing, treatment with fumes or vapors, or any other treatment.

A particularly useful form of heat-sensitive copy-sheet, illustrated in the appended drawing, has a visibly heat-sensitive coating bonded to a thin transparent carrier web. A further opaque protective layer may be applied over the heat-sensitive layer. Heat-converted image areas within the heat-sensitive coating are then viewed through the transparent paper or other carrier. A film-forming binder is normally used with the reactive color-forming components in the heat-sensitive layer. The binder may itself form the carrier web; or the reactants may be supported within a fibrous web structure in the substantial absence of film-forming binder. The reactants are maintained in the required intimate association in physically distinct relationship and in condition for inter-reaction when briefly heated to an appropriate conversion temperature. The copy-sheet is suitable for making direct, high contrast, clear detail, permanent copies of typewritten, printed, and other graphic subject-matter. The copy-sheet does not adhere to nor deface the graphic original or the thermoprinting apparatus. It is stable at normal room and storage temperatures.

The following examples will further illustrate but not limit the invention.

### Example 1

Tetradecyl amine molybdate is first prepared as follows: Tetradecyl amine is first dissolved in an equimolar amount of HCl in aqueous solution, with addition of alcohol and gentle warming where required for complete

2

solution. To the solution thus formed is next added a solution of one-half mol of sodium molybdate, with stirring. The resulting precipitate is removed by filtration, washed to remove sodium chloride, and dried. If desired a further portion may be recovered by evaporation and crystallization. The product is moderately soluble in water. When heated it does not melt, but decomposes and converts from a white to a light brown and then to a gray or greenish-gray color between about 185-240° C.

10 Ten grams of the tetradecyl amine molybdate product is intimately dispersed in acetone by prolonged ball milling. Separately, ten grams of ethyl cellulose and 5 grams of hydroquinone are dissolved in 85 grams of acetone. The two compositions are mixed together and 15 the mixture coated on map overlay tracing paper and dried. The resulting heat-sensitive copy-paper is white in appearance, converting to a reddish brown color when heated in the thermographic copying process or on momentary contact with a metal test bar at a temperature of 130° C.

20 The two compositions may alternatively be separately applied, with intermediate drying. The reactants are intimately associated at the interface between the contiguous coatings. The sheet produces visible but somewhat less distinct copy than is obtainable with single-layer coatings, but pre-reaction of the reactants is avoided.

### Example 2

25 Approximately equal weights of hydroquinone and ethylamine molybdate are mixed together in acetone, the hydroquinone being added to a previously prepared slurry of the ethylamine molybdate formed by ball milling. The mixture is coated on porous paper in the absence of a binder, and dried at room temperature. The initially white sheet is converted to a yellow color when locally heated in the thermographic copying process or by brief contact with the metal test bar at about 100° C.

30 The addition of minor proportions of resinous or polymeric binders to the mixture in acetone permits the formation of firmly bonded heat-sensitive coatings on non-porous films and on dense papers, and increases the temperature at which the color change occurs. For example, the addition to the mixture of Example 2 of small amounts of ethyl cellulose produces a composition which may be 35 coated on non-porous paper and dried to provide a firmly bonded heat-sensitive layer which undergoes permanent change in color on brief contact with the test bar at about 110-120° C.

35 Polystyrene is another resinous binder material useful in the practice of the invention, and coatings prepared with this binder are somewhat more water-resistant than otherwise similar coatings having an ethyl cellulose binder. Polystyrene is conveniently applied from solution in ethyl acetate or in a mixture of acetone and heptane. Other binders in other solvents are also useful, and are preferably so selected as to provide an inert vehicle for the reactants in which one or both of the latter are insoluble.

50 The following tabulation sets forth additional specific

| Example | Reactant A                         | Reactant B                                           | Temp.,<br>°C. | Initial         | Final             |
|---------|------------------------------------|------------------------------------------------------|---------------|-----------------|-------------------|
| 3.....  | tetradecylamine molybdate.         | vanillin.                                            | 80            | white.....      | yellow.           |
| 4.....  | do.....                            | methyl hydroquinone (i.e.,<br>2,5-dihydroxytoluene). | 90            | do.....         | purple-<br>brown. |
| 5.....  | cyclohexylamine molydate.          | hydroquinone.....                                    | 130           | tan.....        | orange-<br>brown. |
| 6.....  | hexamethylene diamine<br>molydate. | do.....                                              | 90            | white.....      | purple-<br>brown. |
| 7.....  | tetradecylamine molybdate.         | 4 - methoxy - 1 - hydroxy-<br>dihydronaphthalene.    | 110           | do.....         | brown.            |
| 8.....  | do.....                            | 2,4-dibromonaphthalene.                              | 100           | do.....         | blue.             |
| 9.....  | do.....                            | catecholacetone condensa-<br>tion polymer.           | 70            | do.....         | brown-<br>black.  |
| 10..... | phenylamine molybdate.....         | hydroquinone.....                                    | 110           | pale<br>yellow. | black.            |

components and combinations which are found useful in the practice of the invention, together with the color change produced and a typical test temperature for color conversion as determined with the heated metal test bar.

The organic amine molybdate is conveniently prepared by the procedure outlined in Example 1, viz. by reaction in aqueous solution of the amine hydrochloride with the stoichiometric quantity of sodium molybdate. Where the product is readily water-soluble, smaller quantities of water are required and suitable precautions must be observed in purifying the material.

The organic amine molybdates are themselves capable of color conversion on heating, at least in some instances. For example, tetradecyl amine molybdate as prepared in Example 1 and coated on filter-paper converts from white to greenish brown when the coated paper is briefly placed in contact with a test bar at 190-200° C.; but corresponding temperatures are likely to cause charring of the paper, and are difficult to attain, in the thermographic copying process. Phenylamine molybdate likewise, when spread in a thin layer on a supporting film or foil and heated slowly to 180-200° C., first converts to a pale green and then to black. Again, certain higher molecular weight organic components tend to increase the temperature requirements unduly; for example a heat-sensitive composition prepared with hydroquinone and octadecyl amine molybdate converts from off-white to blue, but at a test bar temperature well above 150° C. It has previously been found that papers which provide a color change on the test bar at temperatures within the approximate range of 90-150° C., and preferably below about 120° C., are best capable of serving as thermographic copy-papers in commercially available copying apparatus. The present invention makes possible the development of a visible change in the organic amine molybdate composition at a temperature well below the level otherwise required, and well within the range found to be essential for contemporary commercial thermographic copying procedures and apparatus. However the compositions requiring the higher temperatures are useful in sheets, coatings or other structure designed for printing with heated type, or for tracing with a heated stylus, or in other applications requiring a visible change on application of high temperatures.

Molybdates of other organic amines, as well as organic amine tungstates and vanadates, having equivalent properties and characteristics and useful in providing visibly heat-sensitive copying-sheets are contemplated as coming within the ambit of this invention. Other equivalent active reducing agents are likewise contemplated.

What is claimed is as follows:

1. A normally stable heat-sensitive copy-sheet suitable for the thermographic reproduction of differentially radiation-absorptive graphic originals and including a visibly heat-sensitive layer capable of undergoing permanent visible change on brief contact of said copy-sheet with a metal test bar at a temperature within the approximate range of 70° C. to 150° C. and comprising an organic amine molybdate and a reducing agent reactive therewith.

2. A normally stable heat-sensitive copy-sheet suitable for the thermographic reproduction of differentially radiation-absorptive graphic originals and including a visibly heat-sensitive layer capable of undergoing permanent visible change on brief contact of said copy-sheet with a metal test bar at a temperature within the approximate range of 70° C. to 150° C. and comprising an organic amine molybdate and an aromatic hydroxy reducing agent.

3. A normally stable heat-sensitive copy-sheet suitable for the thermographic reproduction of differentially radiation-absorptive graphic originals and including a visibly heat-sensitive layer capable of undergoing permanent

visible change on brief contact of said copy-sheet with a metal test bar at a temperature within the approximate range of 70° C. to 150° C. and comprising an aliphatic amine molybdate and an aromatic hydroxy reducing agent.

5. A normally stable heat-sensitive copy-sheet suitable for the thermographic reproduction of differentially radiation-absorptive graphic originals and including a visibly heat-sensitive layer capable of undergoing permanent visible change on brief contact of said copy-sheet with a metal test bar at a temperature within the approximate range of 70° C. to 150° C. and comprising an aromatic amine molybdate and an aromatic hydroxy reducing agent.

10 6. A normally stable heat-sensitive copy-sheet suitable for the thermographic reproduction of differentially radiation-absorptive graphic originals and including a visibly heat-sensitive layer capable of undergoing permanent visible change on brief contact of said copy-sheet with a metal test bar at a temperature within the approximate range of 70° C. to 150° C. and comprising an aliphatic amine molybdate and a hydroquinone.

15 7. A normally stable heat-sensitive copy-sheet suitable for the thermographic reproduction of differentially radiation-absorptive graphic originals and including a visibly heat-sensitive layer capable of undergoing permanent visible change on brief contact of said copy-sheet with a metal test bar at a temperature within the approximate range of 70° C. to 150° C. and comprising an aromatic amine molybdate and a hydroquinone.

20 8. A high temperature indicator device capable of undergoing permanent visible change when briefly heated to a conversion temperature within the approximate range of 70° C. to 240° C. and including a visibly heat-sensitive layer comprising an organic amine molybdate.

25 9. A normally stable heat-sensitive thermographic copy-sheet capable of undergoing permanent visible change on brief contact with a metal test bar at a temperature within the approximate range of 70° C. to 150° C. and including a layer of reactants maintained in physically distinct relationship and in condition for interaction when thus heated, said reactants comprising a visibly heat-sensitive organic amine molybdate and an aromatic hydroxy reducing agent.

30 10. A normally stable heat-sensitive thermographic copy-sheet capable of undergoing permanent visible change on brief contact with a metal test bar at a temperature within the approximate range of 70° C. to 150° C., said copy-sheet comprising a thin supporting web and a visibly heat-sensitive coating of a composition comprising a film-forming binder, a visibly heat-sensitive organic amine molybdate, and an aromatic hydroxy reducing agent.

35 11. A normally stable heat-sensitive thermographic copy-sheet capable of undergoing permanent visible change on brief contact with a metal test bar at a temperature within the approximate range of 70° C. to 150° C., said copy-sheet comprising a thin supporting web and a visibly heat-sensitive coating of a composition comprising a film-forming binder, tetradecylamine molybdate, and an aromatic hydroxy reducing agent.

40 12. A normally stable heat-sensitive thermographic copy-sheet capable of undergoing permanent visible change on brief contact with a metal test bar at a temperature within the approximate range of 70° C. to 150° C., said copy-sheet comprising a thin supporting web and a visibly heat-sensitive coating of a composition comprising a film-forming binder, tetradecylamine molybdate, and an aromatic hydroxy reducing agent.

#### References Cited in the file of this patent

#### UNITED STATES PATENTS

- |           |                       |               |
|-----------|-----------------------|---------------|
| 1,844,199 | Bicknell et al. ----- | Feb. 9, 1932  |
| 2,663,654 | Miller et al. -----   | Dec. 22, 1953 |
| 2,910,377 | Owen -----            | Oct. 27, 1959 |